

# UNITED STATES PATENT OFFICE.

URLYN CLIFTON TAINTON, OF JOHANNESBURG, TRANSVAAL, SOUTH AFRICA.

## ELECTROLYTIC RECOVERY OF ZINC FROM ORES AND OTHER ZINC-BEARING MATERIALS.

1,210,017.

Specification of Letters Patent. Patented Dec. 26, 1916.

No Drawing.

Application filed August 10, 1915. Serial No. 44,837.

*To all whom it may concern:*

Be it known that I, URLYN CLIFTON TAINTON, B. Sc., a subject of the King of Great Britain, and resident of Johannesburg, 5 Transvaal Province, Union of South Africa, have invented certain new and useful Improvements in the Electrolytic Recovery of Zinc from Ores and other Zinc-Bearing Materials, of which the following is a specification.

10 This invention relates to the electrolytic recovery of zinc from ores and other zinc-bearing materials or substances.

In the specification of a prior Patent Number 1,059,233, dated 15th April, 1913, granted to the present applicant and John Norman Pring jointly, a process is described for extracting zinc by electrolysis from a solution or electrolyte of a specified constitution or 20 composition. According to said specification the requisite solution is obtained by taking or forming a solution of a salt of zinc (for example zinc sulfate) and adding thereto a large proportion of acid (for example sulfuric acid) and a small proportion of a colloid agent (for example gum tragacanth). The deposition of the metallic zinc out of 25 said solution is effected by electrolyzing such solution with a current of high density. 30 The present application appertains to a continuous or cyclic process for the production of such solution directly from ores or other zinc-bearing materials, and to the use of said solution in the aforementioned process for 35 recovering zinc electrolytically.

A feature of the present process is that it can be carried out without loss of acid or accumulation of impurities.

According to the present invention, in a 40 process for the electrolytic extraction of metallic zinc from its ores or other zinc-bearing material, the solution is regenerated by dividing it into two portions, treating fresh ore with one portion thereof to dissolve zinc 45 and neutralize its acid content, and thereafter mixing the neutral solution with the remaining portion for further treatment by electrolysis with a current of high density (for example 50-1000 amperes per square 50 foot) the proportion employed for treating the fresh ore preferably being such that on neutralizing the said content with fresh ore and mixing the resulting neutral solution with the remaining solution, the mixture 55 contains from 5-30% of free acid. The process may often be carried out without the ad-

dition of any colloid, since colloidal silica is usually produced in the solutions by the action of the acid on the ores from which they are formed. A colloid may, however, 65 be added if desired.

One method of carrying out this invention will now be described. The ore or other material from which the zinc is to be extracted is, if requisite, first reduced to such a size as to render the zinc values readily accessible to the solvent. The ore is preferably crushed fairly fine, so as to form with the solution which is to be added a pulp which can be readily agitated. In the case 70 of sulfid and some other zinc ores the material is then roasted, so as to convert the zinc into a form readily soluble in acid. This ore is then treated with an acid, as for example sulfuric acid. This may be effected 75 by percolation, leaching, or agitation, the last method, which is ordinarily applicable, being preferred, as it shortens the time of such treatment. The acid is added in quantity just sufficient to take up the zinc in the 80 ore and leave a neutral solution. This solution is then, if necessary, separated from suspended solid matter, by filtration or settlement, and then acidified by means of a further quantity of acid. When the solution 85 has been separated from the treated ore, the latter is washed with water which is then added to the solution. It is desirable to filter the solution while hot to prevent the zinc sulfate from crystallizing out during filtration. It is preferable so to arrange that the concentration of both zinc and acid in the 90 solution contains a fairly high value, as for example 140 (one hundred and forty) grams of zinc per liter and from 50-300 (fifty to 95 three hundred)—preferably about 75 (seventy-five) grams of free sulfuric acid per liter. The solution is then electrolyzed with insoluble anodes, for example lead sheets, and any suitable cathodes, and with a current of high density, say between 50 (fifty) and 300 (three hundred) amperes to the square foot. The electrolysis is continued 100 until a suitable quantity of zinc has been taken from the solution. This is the case 105 usually when about 60 (sixty) grams per liter have been taken from it, with a corresponding rise in the acid content to say 150 (one hundred and fifty) to 170 (one hundred and seventy) grams of sulfuric 110 acid per liter.

The solution is then regenerated from the

ore in the following way: The solution is divided into two portions such that one portion contains as much free acid as the whole of the original solution did before the electrolysis. This statement may be explained by taking an example. Assuming that the original content of the solution was 75 (seventy-five) grams per liter of free acid and the final content was 150 (one hundred and fifty) grams per liter and the total volume of solution remained the same, then one half of the final solution would be taken. This portion is then kept separate and the remaining portion is used for dissolving out the zinc from a fresh charge of ore. The quantity of ore used is such as will just neutralize all the acid in the portion of the electrolyzed solution taken. When neutralization is practically complete a small quantity of fresh ore is added in order to complete the neutralization and precipitate iron. The solution is then separated from the residue and added to the strongly acid solution which has been retained in the storage vat. When the solution has been separated from the treated ore, the latter is washed with water which is then added to the solution. The acid content of the mixed solution is thereby brought back to its original concentration. The solution may be then again electrolyzed and the operation repeated. Though the presence of iron in the solution does not adversely affect the physical character of the zinc deposited therefrom yet in treating ores for the extraction of zinc by the cyclic process according to the present invention, the iron dissolved in the ore will, if it is not eliminated, gradually increase until it eventually attains a high concentration in the electrolyte and thereby leads to the contamination of the deposited zinc and also tends to lessen the efficiency of the process when the electrolysis is long continued. It is advisable therefore in the present process to precipitate the iron from the solution by the addition of fresh ore.

The quality of the metal deposited under these conditions is very good, and it may be used directly as a galvanizing coating for the protection of iron against corrosion. If, however, the zinc is required in the form of solid metal the cathode used may be of such a nature that the deposit of zinc is readily detached from it, as for example, aluminium, or oiled or graphite-covered copper. The zinc after being detached may be then melted up and cast. Alternatively the zinc may be deposited on thin sheets of zinc foil, which may be then melted without stripping, or a cathode of iron or other material of high fusing point may be used, in which case the zinc deposit may be removed by dipping said cathode in a bath of molten zinc, fused zinc chlorid, et cetera, and the cathode then re-

turned to the depositing vat. If the amount of sulfuric acid consumed by the ore is in excess of that theoretically required, it is desirable to arrange the roasting so that a portion of the sulfur content of the ore is retained in the form of sulfate or basic sulfate. The amount of sulfate so retained may be adjusted by varying the conditions of the roast so as to balance any gain or loss of acid in the dissolving process. <sup>75</sup>

The advantages accruing to the method of treatment which forms the subject matter of this application are:-

(a) It provides a means whereby advantage can be taken of the special benefits <sup>80</sup> which accrue from the use of a high current density, high acid content and the presence of a colloid (*vide* the specification of our prior patent) whereby such solution can be prepared direct from ores and other impure <sup>85</sup> materials without loss of acid or accumulation of impurities.

(b) It is possible to extract metallic zinc directly from the ore, and to deposit such zinc immediately in a form in which it may <sup>90</sup> be used as a protective coating for iron or steel in one operation. This has not been possible on a commercial scale according to known processes.

(c) On account of the high acid content <sup>95</sup> of the solution used for dissolving out the zinc in the ore, the zinc is very rapidly dissolved, and the plant necessary for this operation can be relatively very small; and on account of the high current densities used in <sup>100</sup> the electro-deposition, the depositing plant required is also relatively small, and the number of electrodes, et cetera, required very few.

(d) Under the conditions described it is <sup>105</sup> possible to extract a large amount of zinc from the solution without regeneration of the solution. In this connection it may be stated that this has been one of the main difficulties in the past, as the current efficiency of the zinc electrolysis fell off rapidly as the acid content rose. For this reason, therefore, it was possible to continue the electrolysis only by the provision of special means to prevent the accumulation of acid <sup>110</sup> in the solution, for example, diaphragms, soluble anodes, et cetera. With the solution described, however, a very large amount of zinc can be taken out, as I have found that the accumulation of acid causes no fall in the <sup>115</sup> efficiency. This again leads to a reduction in the size of plant required.

(e) In the case of ores containing iron and manganese, by the neutralization of the solution, and subsequent addition of a small <sup>120</sup> quantity of ore, all iron present may be precipitated. Manganese also, which has proved an insuperable obstacle in the past, owing to the formation of permanganic acid and consequent resolution of the zinc, is con- <sup>125</sup> 130

tinuously eliminated during electrolysis, as I have found that under the conditions described manganese is continuously precipitated at the anodes as manganese dioxide, 5 and can be readily removed from the solution by filtration or settlement. The accumulation of manganese salts in the solution is thereby prevented, and the presence of manganese in an ore exerts, therefore, no deleterious effect whatever upon the quality 10 of the deposits obtained.

(f) In the case of many ores it is possible to vary the quality of the deposits, by making use of the silicic acid formed by the action 15 of the acid solution on the silicates in the ore. This can be used to take the place of the colloid which, as described in the specification of the previous patent, is necessary for the formation of lustrous deposits 20 of zinc.

(g) As the residues are extracted from the solution when neutral, there is no deleterious acid effect on pumps, filters and other plants necessary for handling the solution.

25 The solution prepared according to the present invention, that is, one having a high acid content would be practically useless in any process known in the art except that described in the prior application for patent 30 hereinbefore mentioned as it has not hitherto been possible under ordinary practice to recover metallic zinc from a solution containing a high percentage of free acid and containing also other metals electronegative 35 to zinc.

What I claim as my invention and desire to protect by Letters Patent is:

1. A continuous electrolytic process for the extraction of zinc from a zinc-bearing material which consists in forming therefrom a concentrated solution of a zinc-salt containing an excess of acid, electrolyzing the solution with a current of high density, regenerating the said solution by dividing it into 40 two portions in such proportions that, when the acid in one portion is neutralized by the addition to it of a charge of zinc-bearing material and the resulting solution separated from the residue and mixed with the other portion of the electrolyzed solution which has been retained, the acid-content of the final solution shall be approximately the same as that of the original solution, and then electrolyzing the regenerated solution 45 with a current of high density.

2. A continuous process for the electrolytic extraction of metallic zinc from a zinc-bearing material, which consists in adding sufficient of the zinc-bearing material to an 50 acid to make a neutral solution, separating the neutral solution from the residue, adding an excess of acid and a small proportion of a colloid, electrolyzing said solution by means of a current of high density and thus 55 removing part of the zinc; then removing

the solution now strongly acid and dividing it into two portions, neutralizing one portion by a further addition of zinc-bearing material, separating the neutral solution from the residue, adding the other portion of the removed solution and electrolyzing the acid solution so formed; and thereafter repeating the regenerating and electrolyzing process as described. 70

3. A continuous process for the electrolytic extraction of metallic zinc from a zinc-bearing material which consists in adding sufficient of the zinc-bearing material to an acid to make a neutral solution, separating the neutral solution from the residue, adding an excess of acid, and electrolyzing said solution by means of a current of high density and thus removing part of the zinc; then removing the solution now strongly acid and dividing it into two portions, neutralizing one portion by a further addition of zinc-bearing material, adding a slight excess of zinc-bearing material to the neutral solution to remove any iron or other impurities present, separating the neutral solution 80 from the residue, adding the other portion of the removed solution, and electrolyzing the acid solution so formed; and thereafter repeating the regenerating and electrolyzing process as described. 85

4. A continuous process for the electrolytic extraction of metallic zinc from a zinc-bearing material, which consists in adding sufficient of the zinc-bearing material to an acid to make a neutral solution containing the colloid required in the production of smooth zinc deposits, separating the neutral solution from the residue, adding an excess of acid, and electrolyzing said solution by means of a current of high density and thus removing part of the zinc; then removing the solution now strongly acid and dividing it into two portions, neutralizing one portion by a further addition of zinc-bearing material, separating the neutral solution from the residue, adding the other portion of the removed solution, and electrolyzing the acid solution so formed; and thereafter repeating the regenerating and electrolyzing process as described. 95

5. A continuous electrolytic process for the extraction of zinc from its ores which consists in forming therefrom a concentrated solution of a zinc-salt containing from 50-300 grams of free acid per liter, 100 electrolyzing the solution with a current of high density, regenerating the said solution by dividing it into two parts in such proportions that, when the acid in one portion is neutralized by the addition to it of 105 a charge of ore and the resulting solution separated from the residue and mixed with the other portion of the neutralized solution which has been retained, the acid content of the final solution shall be approxi- 110 115 120 125 130

- 4
- mately the same as that of the original solution, and then electrolyzing the regenerated solution with a current of high density.
- 5 6. A continuous process for the electrolytic extraction of zinc from its ores which consists in adding sufficient of the ore to an acid to make a neutral solution, separating the neutral solution from the residue, adding an excess of from 50-300 grams of free acid per liter and a small proportion of a colloid, electrolyzing said solution by means of a current of high density and thus removing part of the zinc; then removing the solution now strongly acid and dividing it into two portions, neutralizing one portion by a further addition of ore, separating the neutral solution from the residue, adding the other portion of the removed solution, and
- 10 15 20 25 30 35 40
- electrolyzing the acid solution so formed; and thereafter repeating the regenerating and electrolyzing process as described.
7. A continuous process for the electrolytic extraction of metallic zinc from its ores which consists in adding sufficient of the ore to an acid to make a neutral solution, separating the neutral solution from the residue, adding an excess of from 50-300 grams of free acid per liter, and electrolyzing said solution by means of a current of high density and thus removing part of the zinc; then removing the solution now strongly acid and dividing it into two portions, neutralizing one portion by a further addition of ore, adding a slight excess of ore to the neutral solution to remove any iron or other impurities present, separating the neutral solution from the residue, adding the other portion of the removed solution, and electrolyzing the acid solution so formed; and thereafter repeating the regenerating and electrolyzing process as described.
8. A continuous process for the electrolytic extraction of metallic zinc from its ores which consists in adding sufficient of the ore to an acid to make a neutral solution containing the colloid required in the production of smooth zinc deposits, separating the neutral solution from the residue, adding an excess of from 50-300 grams of free acid per liter and electrolyzing said solution by means of a current of high density and thus removing part of the zinc; then removing the solution now strongly acid and dividing it into two portions, neutralizing one portion by a further addition of ore, separating the neutral solution from the residue, adding the other portion of the removed solution and electrolyzing the acid solution so formed; and thereafter repeating the regenerating and electrolyzing process as described.
9. In a continuous electrolytic process for the extraction of zinc from a zinc-bearing material in which a solution of a zinc salt containing an excess of acid is electrolyzed with a current of high density, the step of regenerating the solution by dividing the same into two portions in such proportions that when the acid in one portion is neutralized by the addition thereto of a charge of zinc-bearing material and the resulting solution separated from the residue and mixed with the other portion of said electrolyzed solution which has been retained, the acid-content of the final solution is approximately the same as that of the original solution.
- In testimony whereof I have signed my name to this specification in the presence of two subscribing witnesses.
- URLYN CLIFTON TAINTON.
- Witnesses:
- ARTHUR THOMPSON,  
VIOLET WELLS.